

# United States Patent

Blumbergs et al.

[15] 3,691,139

[45] Sept. 12, 1972

[54] **SODIUM MALEATE  
PEROXYHYDRATE**

[72] Inventors: **John H. Blumbergs**, Highland Park;  
**Paul R. Mucenieks**, Trenton, both of  
N.J.

[73] Assignee: **FMC Corporation**, New York,  
N.Y.

[22] Filed: **June 18, 1970**

[21] Appl. No.: **47,551**

[52] U.S. Cl. ....**260/78.4 R**, 252/94, 260/78.5 T

[51] Int. Cl. ....**C08f 27/04**

[58] Field of Search.....**260/78.4 R, 78.5 T**

[56] **References Cited**

**UNITED STATES PATENTS**

3,496,150 2/1970 **Kropp.....260/78.4**

*Primary Examiner*—Joseph L. Schofer

*Assistant Examiner*—John Kight, III

*Attorney*—Milton Zucker, Frank Ianno, Eugene G. Seems and Pauline Newman

[57] **ABSTRACT**

Sodium maleate peroxyhydrate, useful as a combined detergent builder and bleach, is described, together with its preparation.

**2 Claims, No Drawings**

## SODIUM MALEATE PEROXYHYDRATE

## BACKGROUND OF THE INVENTION

The commonly used detergent compositions include soaps and synthetic detergents, mixed with compounds known as builders, which act both to improve the detergent power of the primary detergents, and to reduce the cost of the overall compositions. The inorganic polyphosphates, such as sodium and potassium tripolyphosphate, have been almost universally used as the bulk of the builder constituents in such compositions. However, there has been a growing resistance to the use of polyphosphates, on the ground that they induce the build-up of undesirable vegetation in waters into which the detergents' wastes are eventually discharged, and there has been a growing demand for detergent builders which would not cause this difficulty. Any such detergent builder must, of course, have optimum economics, and should not produce different environmental hazards than do the phosphates.

Many such builders have been suggested, but all have substantial disadvantages. Nitrilotriacetic acid, which is currently being used commercially as a substitute for phosphates, is both more expensive and potentially dangerous, in that it can keep quantities of heavy metals in solution in water. Other available builders are either much more costly, or have other serious drawbacks.

A potentially interesting group of possible detergent builders comprises the alkali metal salts of poly(carboxylic acid)s as described in Diehl U.S. Pat. No. 3,308,067 issued Mar. 7, 1967. This patent describes the use, as builders, of the water-soluble salts of poly(carboxylic acid)s, the simplest and least expensive of which are the sodium salts of various poly(maleic acid)s.

The least expensive of these salts is sodium polymaleate. It has not, however, come into commercial use because of its slow solubility in cold water, and because it tends to cause caking in mixed detergent formulations.

In copending application of Blumbergs and MacKellar, titled "Sodium polymaleate hydrate," filed simultaneously herewith, there is described a hydrate of sodium polymaleate with a mol of water for each sodium atom in the polymer, which is both more rapidly soluble in cold water and which does not cause caking in mixed detergent formulations.

## STATEMENT OF THE INVENTION

We have discovered that sodium polymaleate will form a peroxyhydrate with hydrogen peroxide and water, in which there is present for each sodium atom a mol of hydrogen peroxide plus water. The product is prepared by suspending sodium polymaleate in an inert liquid carrier, and exposing it to hydrogen peroxide, preferably aqueous, to get the desired product, and filtering and drying the peroxyhydrate. The product is as rapidly soluble and as noncaking as sodium polymaleate hydrate, and is also useful in contributing bleaching power to a mixed detergent.

## DETAILED DESCRIPTION OF THE INVENTION

Sodium polymaleate, useful as a detergent builder, may be prepared as described in Berry U.S. Pat. No.

3,359,246 or as described in the copending Blumbergs et al. application titled "Preparation of sodium polymaleate," mailed to the Patent Office on May 28, 1970 now U.S. Pat. No. 3,637,609. The product is a homopolymer with the structure



15 where  $n$  is at least 3, and may be as high as is permitted by solubility consideration, generally not above about 500; most advantageously, the molecular weight is in the 2,500 to 25,000 range. The product dissolves readily in hot water when in a typical built detergent, but so 20 slowly in cold water that it is not useful in cold-water laundering. Moreover, there is a tendency to cause caking in some mixed detergent formulations. These disadvantages are overcome by forming the hydrate in which a mol of water is bound to each sodium atom.

25 We have found that the water in such a hydrate can be partially or completely replaced by hydrogen peroxide without losing the advantages of the hydrated product over the anhydrous product, while at the same time adding to the product active oxygen which is a useful bleach in detergent formulations.

By using 100 percent hydrogen peroxide and anhydrous sodium polymaleate as the starting compositions, a product can be obtained with 29.8 percent of  $\text{H}_2\text{O}_2$  (14 percent active oxygen), corresponding to a 30 mol of  $\text{H}_2\text{O}_2$  per atom of sodium. However, the high cost of 100 percent hydrogen peroxide, and the dangers inherent in handling it, make this product 35 economically undesirable. Material containing equal molar percentages of water and peroxide is much easier and more economical to prepare, and contains enough active oxygen (7.8 percent) to serve the purpose of adding a powerful bleach to a mixed detergent composition. We may, of course, operate over the whole range 40 of peroxide-to-water ratios, and still get some bleaching value.

The method we use to prepare our new peroxyhydrates is to suspend the sodium polymaleate in a 45 liquid medium which is a nonsolvent for the sodium polymaleate and is inert to the hydrogen peroxide, slowly add the hydrogen peroxide and water in the desired ratio, while agitating, to form the peroxyhydrate, and then filter the peroxyhydrate from the medium.

50 The sodium polymaleate used should preferably be anhydrous, but water can be compensated for by using more hydrogen peroxide or a more concentrated solution. The hydrogen peroxide may be employed in any desired concentration, depending on the ratio of peroxide wanted in the peroxyhydrate; it will add on in the 55 same ratio as present in the reaction medium.

The reaction temperatures are a matter of choice; high temperatures favor fast reaction and peroxide decomposition, low temperatures slow the reaction. 60 We prefer to operate at 30°C. or lower for economic reasons, and for the same reasons prefer not to refrigerate.

Reaction times depend on temperature and agitation rates. Generally about 30 minutes are required for addition, and at ordinary ambient temperatures 1 hour overall is sufficient to ensure complete reaction.

The reaction medium can be any volatile liquid which is a nonsolvent for the polymer salt, and does not react with hydrogen peroxide under conditions of use. Ability to azeotrope excess water is useful. The carriers of choice are aliphatic, aromatic or alicyclic hydrocarbons and halogenated hydrocarbons boiling between 40° and 120°C, e.g., chloroform, carbon tetrachloride, methylene chloride, the various perfluorocarbons, benzene, toluene, cyclohexane and petroleum distillates. These liquids all can be easily separated from the insoluble peroxyhydrates, and the small amounts adhering can be readily evaporated.

#### SPECIFIC EXAMPLES OF THE INVENTION

The following examples of the invention are given by way of illustration, and not by way of limitation.

##### EXAMPLE 1

In a 250 ml beaker were placed 16 g of sodium polymaleate powder, -100 mesh, and 50 ml of toluene. A magnetic stirrer was used to stir the slurry, while 5.3 g of 70 percent hydrogen peroxide were added dropwise. Some lump formation was observed. The lumps were crushed and addition of  $H_2O_2$  continued. Total addition time was 35 minutes. The slurry was left overnight, then filtered and dried in a circulating air at 55°C. There were obtained 16.9 g of white solids having an active oxygen content of 5.35 percent by weight.

##### EXAMPLE 2

The same as Example 1, only 50 ml of chloroform were used in place of toluene. There were obtained 17.2 g of white solids, having an active oxygen content of 6.35 percent.

##### EXAMPLE 3

The same as Example 1, only 50 ml of n-heptane were used in place of toluene. There were obtained 17.0 g of white solids having an active oxygen content of 6.12 percent.

##### EXAMPLE 4

The same as Example 1, only 50 ml of cyclohexane were used in place of toluene. There were obtained 17.3 g of white solids having an active oxygen content of 5.75 percent.

##### EXAMPLE 5

Sodium polymaleate, 80 g (0.5 mol), was placed in a 1-liter, three-neck round-bottom flask, supplied with a laboratory stirrer, condenser and Dean-Stark trap for collecting water. The flask was charged with 500 ml of

toluene, which was boiled for 3 hours under a slight reflux to remove all the moisture from the sodium polymaleate sample.

The flask content was then cooled to 10°C in an ice bath and 27.0 g (0.55 mol) of 70%  $H_2O_2$  were slowly added with good stirring. Addition time was 35 minutes. The slurry was then stirred for an additional hour, was filtered and the solids were dried on Rinco under reduced pressure to remove the toluene solvent. There were obtained 102 g of white solids, having an active oxygen content of 8.3 percent as determined by iodometric titrations.

#### EXAMPLE 6

The sodium polymaleate perhydrate samples were placed in glass jars with vented caps and were stored at 55°C for 3 days to check the stability of this compound.

The active oxygen content was measured before and after the storage. The data are listed in Table 1.

TABLE 1

#### Storage Stability of Sodium Polymaleate Perhydrate

| Sample No. | Storage Time (Days) | Storage Temp. (°C) | % Active Oxygen Before | % Active Oxygen After |
|------------|---------------------|--------------------|------------------------|-----------------------|
| 1          | 3                   | 55-56              | 5.35                   | 5.12                  |
| 2          | 3                   | 55-56              | 6.35                   | 5.91                  |
| 3          | 3                   | 55-56              | 6.12                   | 6.03                  |
| 4          | 3                   | 55-56              | 5.75                   | 5.42                  |
| 5          | 3                   | 55-56              | 8.30                   | 8.12                  |

The data indicate that the sodium polymaleate perhydrate compound has sufficient storage stability to be used as a detergent builder and a bleach. Under the above mentioned accelerated test conditions, only a slight drop in active oxygen content was noticed.

Obviously, the examples can be multiplied indefinitely without departing from the invention as defined in the claims.

We claim:

1. Solid, noncaking sodium polymaleate peroxyhydrate containing one mol of hydrogen peroxide plus water of crystallization for each atom of sodium in the polymaleate.

2. The method of making solid non-caking sodium polymaleate peroxyhydrate containing 1 mol of hydrogen peroxide plus water of crystallization for each atom of sodium in the polymaleate, which comprises heating sodium polymaleate which is at least partially anhydrous suspended in a liquid nonsolvent therefor which is nonreactive with hydrogen, with hydrogen peroxide in sufficient quantity to yield a mol of hydrogen peroxide plus water per atom of sodium in the polymaleate for a sufficient time to complete pick-up of the hydrogen peroxide by the sodium polymaleate, and separating the peroxyhydrate from the carrier.

\* \* \* \* \*